

Sept. 8, 1931.

S. E. SEAMAN

1,822,174

# METHOD FOR THE TREATMENT OF CELLULOSE AND PRODUCT RESULTING THEREFROM

Filed July 3, 1926

2 Sheets-Sheet 1



Inventor  
Stewart E. Seaman  
by Roberto, Cushman & Woodberry  
Att'y's

Sept. 8, 1931.

S. E. SEAMAN

1,822,174

METHOD FOR THE TREATMENT OF CELLULOSE AND PRODUCT RESULTING THEREFROM.

Filed July 3, 1926

2 Sheets-Sheet 2



Fig. 2



Fig. 3



Fig. 4

Inventor  
Stewart E. Seaman

By Roberta Cushman & Woodberry.

Att'y's

## UNITED STATES PATENT OFFICE

STEWART E. SEAMAN, OF BANGOR, MAINE, ASSIGNOR TO EASTERN MANUFACTURING COMPANY, OF SOUTH BREWER, MAINE, A CORPORATION OF MASSACHUSETTS

METHOD FOR THE TREATMENT OF CELLULOSE AND PRODUCT RESULTING THEREFROM

Application filed July 3, 1926. Serial No. 120,372.

This invention relates to a method for the treatment of cellulosic materials made from wood to provide chemical and physical condition suitable for subsequent chemical conversions (especially esterification) and to products resulting from the application of the invention.

Owing to the unique characteristics of cotton fibre, (including the fact of its initial purity, its relatively long fibrous structure, its preliminary resistance to chemical reagents and physical manipulations, sufficient to permit of cleaning and purifying the same without profound alteration, and also the availability of the product in commercial quantities) it has heretofore been considered as a standard and preferred raw material for the manufacture of cellulosic derivatives such as nitrocelluloses and the like, in which control of the conversion reactions, certainty of the final chemical composition and uniformity of physical properties of the resulting product are essential elements.

However, when contrasted with the cost of other sources of cellulosic materials, cotton has been relatively expensive. Consequently, numerous efforts have been made to render such cheaper materials available for the purpose of chemical conversion into various cellulosic derivatives. In this endeavor, wood has usually been the primary source considered, or some of the by-products of wood such as sawdust, or in a few instances cellulosic substances of other derivation.

Without enumerating the various courses which such efforts have taken or the measure of success or failure by which they have been ultimately attended, it is here sufficient to state that in general they did not recognize, or they disregarded those chemical and physical characteristics of cellulosic materials or fibres which facilitate or are essential to the subsequent reactions required, leading to the final result to be accomplished. To such extent as these characteristics have been imperfectly understood and provided for in the preliminary steps, procedures and treatments of the prior art have not produced a suitable cellulose for purposes of converting it into its derivatives.

In this connection it is to be observed that while cotton possesses the qualities above set forth to recommend it for chemical treatment, the raw cotton fibre itself is not, in the first instance, susceptible to a ready and uniform conversion into cellulosic derivatives. On the contrary, it requires the preliminary removal of impurities, including a superficial film consisting of a more resistant wax-like substance which covers and effectively protects the cellulosic body portion of the individual fibre. In order to adequately effect this removal, the cotton must be subjected to a suitable treatment, sufficiently active to remove this outer waxy layer. In the course of such treatment, the inner cellulosic substance is unavoidably reacted upon and, in the use of aqueous solutions, is invariably changed. This will occur as a condition inherent to such processes, even though the utmost precautions and care are taken to avoid further action by the reagents or by the mechanical treatments employed, before removal of the wax-like coating has been accomplished.

A similar condition is presented by other cellulosic materials, though usually such materials ordinarily present further problems. In the consideration of cellulosic raw materials, such as wood pulp generally, for purposes of esterification it is apparent that a more intensive purification treatment is required and by whatsoever process employed reduced to the condition of a pulp or subsequently purified to the degree desirable for esterification or like purposes.

It is to be observed and emphasized as an inherent part of the general concept of the present invention that, while the chemical condition of the cellulosic material to be reacted upon is of fundamental importance, the physical characteristics which are manifest in the esterification process are equally as important if not in actual practice functionally more controlling. For example, attention is directed to the specific qualifications, that in order for the esterifying reagent to react uniformly upon the individual cellulosic fibres, it must come into intimate and uniform contact therewith. It must also

effect such contact rapidly in order that the time of reaction upon all portions of the charge of the cellulose base under treatment may be approximately the same. Otherwise, since the composition of the cellulosic derivative actually produced (as with the nitrates) is a direct function of the time of reaction, those portions which are first brought into contact with the esterifying agent may be over-converted, relative to those acted upon afterwards.

This would imply a substantially instantaneous penetration of the esterifying reagent upon and into each and every portion and particle of the cellulosic material under treatment. Incidental to such penetration, there is also involved the simultaneous displacement of entrained volumes of air or other gaseous inclusions, as well as the superficially adsorbed gaseous components which may be associated with the surfaces of the individual cellulosic fibres. Moreover, the reagent must also reach all parts of the cellulosic substance in quantities sufficient to bring about the desired conversion.

In this aspect of the physical conditions of the esterifying reaction, the course of the chemical reaction or reactions again becomes predominant. That is to say, upon the initial contact of the cellulose body with the esterifying reagent, an apparent gelatinization may take place, inhibiting further penetration of reacting agents. This retards or inhibits further penetration of the esterifying reagent into the cellulosic material and therefore may not only cause the formation of successive layers of cellulose structure characterized by successively reduced degrees of esterification from the outer surface to the center but may leave the central portions of the cellulose aggregates entirely unaffected thereby.

It is therefore an object of this invention to provide a mode of treatment for cellulosic material (other than cotton) for the purpose of reducing the same to both a physical condition and chemical state closely associated with the subsequent conversion of the same into esters or other derivatives, uniformly, and upon a commercial scale. Further and more specific objects of the invention will be manifest from the following disclosure.

The procedure involving the subject matter of this invention includes in general terms a preliminary reduction of the cellulosic material from the condition in which it is usually found in nature to the condition of a pulp, retaining the fibrous structure thereof so far as may be consistent with an adequate opening up of the raw material, removing the reagents and other materials which are entrained in or associated with the cellulosic portion and may be regarded as impurities, putting the pulp thus produced into any con-

venient form, a portion of the water being removed therefrom, then forming the fibrous mass into separated aggregates of a predetermined order of size or sizes, (without substantially compacting or consolidating the same) and finally drying the resulting mass of fibrous cellulosic aggregates.

More specifically, the invention will be described in its relationship to the preparation of wood cellulose by the sulfite process, resulting in a pulp of a relatively high degree of alpha cellulose. This is followed by a second-stage treatment of the pulp generally characterized by reagents (such as alkaline solutions, with or without alkaline metal reactive compounds of sulfur) effective to remove further impurities without appreciable detrimental action upon the cellulosic content, and finally partially dehydrating the pulp and subjecting it preferably to a succession of finely gauged and closely spaced picker teeth by which the individual groups of fibres are caught and rent apart (without appreciable disruption of the fibres themselves) into small tufts or aggregates. These aggregates are more or less uniform in size or volume and are characterized by a high alpha cellulose content and substantially free from resins and other reaction-inhibiting substances, in such condition as to facilitate penetration by the fibre-wetting liquids without entrapped air or liberated gases of reaction to a commercially detrimental degree.

The physical condition of the fibrous aggregates so produced may be attributed to the procedure of engaging the fibres with extremely fine points at suitably spaced intervals and plucking the fibres engaged by one point and those more or less firmly intertwined with them from those engaged by an adjacent point (and the fibres intertwined with them) without destroying the length of individual fibres and at the same time without detrimentally compacting such clusters of fibres together. It is, nevertheless, believed that the picking points do compact the fibres immediately engaged thereby to a sufficient extent to promote the interlocking arrangement and to thereby create an integrity of the aggregate of fibres which in experience is found to be persistently preserved throughout such subsequent handling as may be necessary in fibre form for baling, storage, etc.

While the ultimate size or volume of such aggregates may be controlled and varied at will, the number of fibres which each aggregate contains will necessarily be varied. Hence, what may be termed the "fibre density" of the separate tufts or aggregates produced by the present invention may be correspondingly controlled and varied (in the maximum size) to accommodate the product to specific requirements of the subsequent conversions to which it is to be subjected. In actual experience, for example in nitrat-

ing the product with mixed acid, it has been found that when the aggregates are approximately of the size of mustard seed, weighing approximately 1 milligram or less and containing approximately 40,000 fibres or less, a satisfactory nitration thereof may be accomplished and a uniform and stable nitrated product is obtained.

A typical succession of steps leading to 10 a product of the desired chemical and physical characteristics with respect to a subsequent conversion, as to nitrocellulose will now be described, reference being had to the accompanying drawings, in which:

15 Fig. 1 is a diagrammatic representation of a series of apparatus used, and to be considered as in the nature of a flow sheet;

Fig. 2 is a side elevation more in detail of the picker element of the apparatus;

20 Fig. 3 is a front view of the picker teeth rollers; and

Fig. 4 is an enlarged view of the picker teeth per se.

Referring now to Fig. 1 of the drawings, 25 numeral 1 indicates the raw material in convenient form, 2 a conveyor leading to the hopper of shredder 3 which stands above the manhole 4 of rotary digester 5. The latter is mounted above the washing vat 6, dis-

30 posed as to transfer the charge from 5 to vat 6. Tank 6 has an outlet shown at 7 into bleach tank 8 from which conduit 9 leads through valve 11 and pump 12 to a thickener 13. This may be of other form but is shown

35 as comprising screen roll 14 and couch roll 15, from which the pulp may be delivered over chute 16 to conveyor 17 leading to squeeze rolls 18, followed by conveyor 21, 22, feed rolls 23, and picker 24. The latter may

40 be of any desired type and delivers through chute 26 to tower 28 having latticework 29 or similar retarding means for catching the product delivered to it and permitting it to fall on conveyor 31 leading to the picker 33.

45 The latter comprises a central drum 34 mounted for rotation on trunnions 35 and having parallel and adjacent to the upper arc of its periphery a series of smaller picker roll workers shown as 36, 37, 38, 39, 40, 41 and 42

50 conveniently spaced. The larger drum or cylinder 34 (see Figs. 2 and 3) is provided with teeth 43 properly formed along the margin of a continuous metal strip 44 as shown in Fig. 4. This strip may be mounted in helical

55 grooves in the surface of the cylinder 34, and firmly seated therein and peened in position. The adjacent rows of teeth 45 may be spaced apart by varying distances but are in any event relatively close together, as shown in

60 Fig. 3 (by which satisfactory results have been obtained using 22 rows to the linear inch). The smaller picker rolls 36 to 42 inclusive may be similarly provided with picker teeth 46 in rows 47 spaced apart to correspond

65 to the rows upon cylinder 34.

The roll 34 and peripheral surfaces or teeth of the smaller picker rolls (36 to 42) may be adjustably spaced apart to correspond to the specific requirements of operation desired. The teeth 46 on the smaller picker rolls may 70 also be differently spaced apart. For example, the teeth upon the strips used in picker roll 36 may be of the order of 10 to the linear inch while those on succeeding rolls 37 to 42 may be successively more closely 75 spaced, so that the teeth on picker roll 42 will be 26 or more to the linear inch. Again, it should be understood that these rows or the teeth thereon may be differently spaced, depending upon the nature of material oper- 80 ated upon and the final result desired.

The picker 33 is provided with a cylindrical brush 48 having wire or other bristles 49 which lightly contact with the surface of roll 34 and are suitably mounted for rotation 85 as upon trunnions at 50 and driven by pulley 51. Below the brush is provided a dryer apron 52 leading through a drying chamber 53 to a chute 54 which in turn exists to a baling or compressing chamber 55 in which 90 a piston 56 may be slidably mounted and eccentrically connected by driving rod 57 to the eccentric 58. The exit to the baling chamber may be at 59 from which the bales of compressed pulp may be withdrawn. 95

In operation the raw material may be pulp which has been obtained by methods now known and would be ordinarily selected with a view to the relative purity (with respect to the cellulosic content) which such pulps manifest and to the minimum of degenerated fibre. Again such preliminary treatment may be varied in view of the subsequent operations to which the pulp is to be subjected. As an example, in one application of the invention now to be described, a suitable wood such as spruce may be first reduced to chips and then digested in accordance with the usual bisulfite treatment, which is preferably diminished in duration or in intensity 100 of action or both to constitute a "raw cook", —or even somewhat less than what, for purposes of paper making, would be regarded as a suitable "raw cook", —then washed and subjected to a bleaching treatment if desired. 110

The material (wood pulp 1 as obtained above) is fed onto the conveyor belt 2 by which it is delivered to the shredder 3. It is torn apart and discharged through the manhole 4 into digester 5. Here it is treated 120 with an alkaline solution preferably containing a reactive compound of sulfur, such as sodium sulfite. This solution may be of a concentration of approximately 3% by weight of reagent materials, but preferably 125 contains substantially equal parts of the caustic soda and of bisulfite (see copending application of C. A. Blodgett and H. H. Hanson, Serial No. 87,806, filed February 12, 1926). 130



2. A process for the preparation of cellulosic materials especially suitable for esterification purposes which comprises reducing wood to the condition of a fibrous pulp, purifying the same by removal of impurities contained therein, conducting and controlling said treatment so as to alter the physical and chemical properties of the cellulose, to a condition adapted for rapid wetting of the same 10 by esterifying reagents, partially removing moisture, and forming the same into fibre aggregates of a predetermined order of size, by the operation of picking, and finally drying.

15 3. A process for treating cellulose from wood, comprising purifying the same with an alkaline solution, washing the thus treated pulp free from extraneous materials, bleaching, separating the bleaching liquor therefrom, removing excess water, passing the pulp thus obtained through a succession of picker rolls having teeth thereon closely spaced and in closely arranged rows, to form cellulosic fiber aggregates of approximately 20 one milligram in weight or less and containing an approximate maximum of forty thousand individual fibers per aggregate, and finally drying.

30 4. A process for treating cellulose from wood, comprising purifying the same with an alkaline solution containing sodium sulfite, washing the thus treated pulp free from extraneous materials, bleaching, separating the 35 bleaching liquor therefrom, removing excess water, passing the pulp thus obtained through a succession of picker rolls having teeth thereon closely spaced and in closely arranged rows, to form cellulosic aggregates 40 of approximately one milligram in weight or less and containing an approximate maximum of forty thousand individual fibers per aggregate, and finally drying.

45 5. A cellulosic product consisting essentially of separated, purified, independent wood cellulose fibers, characterized by being assembled into independent aggregates or clusters, the individual fibers of the same being in interlocking engagement with each 50 other and radiating therefrom in mutually spaced relationship to form independent highly absorbent masses.

55 6. An aggregate or cluster of purified, separated wood cellulose fibers, said fibers contacting with each other in interlocking engagement, and radiating freely in mutually spaced relationship therefrom to form a highly absorbent mass.

60 7. An aggregate or cluster of purified, separated wood cellulose fibers, said fibers contacting with each other in interlocking engagement, and radiating freely in mutually spaced relationship therefrom to form a 65 highly absorbent mass, said aggregate or

cluster being characterized by containing less than 40,000 fibers.

8. An aggregate or cluster of purified, separated wood cellulose fibers, said fibers contacting with each other in interlocking engagement, and radiating freely in mutually spaced relationship therefrom to form a highly absorbent mass, said aggregate or cluster being characterized by weighing approximately a milligram or less. 70 75

Signed by me at Boston, Massachusetts, this 26th day of June, 1926.

STEWART E. SEAMAN.